

May 12, 1942.

T. G. FINZEL

2,282,568

CELLULOOSIC STRUCTURE AND METHOD FOR PREPARING SAME

Filed Oct. 5, 1938



*Fig. 1*



*Fig. 2*

*Theron G. Finzel* INVENTOR

BY *Zonis Attache*  
ATTORNEY

## UNITED STATES PATENT OFFICE

2,282,568

CELLULOSIC STRUCTURE AND METHOD  
FOR PREPARING SAMETHERON G. FINZEL, KENMORE, N. Y., assignor to  
E. I. du Pont de Nemours & Company, Wil-  
mington, Del., a corporation of Delaware

Application October 5, 1938, Serial No. 233,484

26 Claims. (Cl. 8—129)

This invention relates to artificial fibers, filaments or the like and yarns, threads, cords or the like composed of artificial fibers and filaments, and methods for producing same. More particularly, it relates to threads, yarns, cords or the like composed of artificial fibers, filaments, or the like having a unique, random crimp and improved methods for producing such structures. The invention is particularly applicable and has exceptional utility in the formation of curls and crimps in thermoplastic cellulosic filaments and yarns.

It has been recognized for some time that the warmth of wool is due mainly to the air spaces entrapped between adjacent fibers and also due to the ability of these fibers to maintain such air spaces even after the fabrics composed thereof have been subjected to water-wetting and/or mechanical forces. The ability of wool in this regard is largely traceable to the decided crimp inherently present in wool, particularly of the finer high grade types. In contrast yarns, composed of artificial fibers or filaments such as cellulose acetate rayon, viscose rayon, or cuprammonium rayon, by virtue of the fact that they normally are spun under tension, are silk-like and possess straight filaments which are devoid of any crimp or curl. Accordingly, it has been reasoned logically that in order to impart a wool-like warmth characteristic to artificial fibers, it would be necessary to insert a curl or crimp in the same.

Numerous methods for imparting curls or crimps to yarns composed of artificial filaments have been proposed prior to this invention. However, great difficulty has attended the impartation of a curl or crimp which will be substantially permanently retained by the filaments without objectionably degrading the same. Prior methods for crimping or curling yarns and filaments have failed due to the impartation of the curls and crimps in a state of stress and strain and consequently an abnormal or unstable condition. Under such conditions, of course, the permanency of the crimp is not altogether satisfactory, since naturally the crimped yarn tends to revert to a normal straight yarn in order to relieve the stress and strain.

An object of this invention is to provide a crimped yarn composed of crimped artificial filaments or fibers in which the crimped condition represents essentially the natural or normal state, free from stress and strain, so that change of such kink or crimp to a straight condition repre-

sents to a certain extent a condition of stress and strain.

Another object is to provide a yarn composed of crimped, artificial filaments in which the crimp is relatively more permanent and less easily removed than a crimp imparted by mechanical means.

A further object is to provide a yarn composed of crimped, artificial filaments characterized by a deep, random, and irregular crimp, i. e., the curvature, sharpness, and amplitude of successive kinks are irregular and some of the different kinks lie in different planes with respect to each other and without any definite pattern.

A further object is to provide from these crimped, artificial filament-containing yarns textile fabrics, particularly of the pile fabric type, that possess an increased fullness.

A still further object is to provide the crimped yarn of the invention in the form of a continuous filament yarn.

A specific object is to provide a thermoplastic, cellulosic yarn having the permanency and type of crimp described in the above objectives.

A more specific object of the invention is to provide a relatively effective and economical procedure of accomplishing the above objects.

Other objects of the invention will appear hereinafter.

30 The crimped yarn of the invention is prepared by a process comprising impregnating a yarn composed of artificial fibers or filaments with a substance capable of vaporizing rapidly when heated to a suitable temperature below the melting point of the yarn, suddenly contacting the impregnated yarn, while maintaining the same free from tension and thus permitting it to shrink freely, into a hot bath consisting of a liquid non-solvent for the yarn and thereby removing rapidly substantially all the vaporizable substance from the yarn whereby a crimp is simultaneously imparted to the filaments which crimp is also exhibited by the yarn.

45 The invention will be more clearly apparent by reference to the following detailed description taken in connection with the accompanying illustrations, in which;

Figure 1 is a diagrammatic illustration of one form of apparatus adapted to carry out the process of this invention.

Figure 2 is a highly magnified view showing a yarn which has been subjected to the crimping process of this invention.

In the illustrations reference numeral 5 designates a cake of yarn composed of artificial

filaments which has been impregnated or conditioned with a vaporizable liquid in a manner hereinafter to be described. The yarn 6 is removed from the bobbin 5 by means of positively driven feed rolls 7, 8, and 9. The thread passes from the feed rolls into a tank 10 containing a liquid high boiling non-solvent for the yarns. The liquid is maintained at a temperature below the melting point of the yarn but at least 30° above the boiling point of the vaporizable liquid with which the yarn has been treated. The yarn 6 is removed from the tank 10 by means of positively driven feed rolls 11, 12, and 13. The yarn, during its contact with the hot liquid is maintained free from any tension so as to permit free shrinkage of the yarn. A large number of deep, irregular crimps projecting in all directions is imparted to the filaments of the yarn. The speed of feed rolls 7, 8, and 9 and the speed of feed rolls 11, 12, and 13 may be so adjusted as to continuously maintain a section of the yarn in free coils within the hot liquid. The yarn is passed from feed rolls 11, 12, and 13 into a collecting can 14 or the like where it is collected in loose coils without imparting tension thereto.

After the yarn 6 has been subject to the above-described crimping operation, the filaments 6a will exhibit individual crimps which are out of phase with each other as shown in Figure 2.

In the preferred embodiment of the invention a substantially untwisted thermoplastic cellulosic yarn composed of a plurality of filaments is treated so as to give the filaments deep, random, and irregular crimps that represent a normal, stable condition. This may be accomplished in the following manner. The thermoplastic yarn is impregnated or conditioned with a vaporizable liquid having an atmospheric boiling point at least 30° C. lower than the temperature of the hot crimping bath. In the case of a relatively water-soluble vaporizable liquid, including water, the thermoplastic yarn is conditioned in contact with the saturated vapors thereof until the yarn has sorbed an amount equal to but not exceeding a saturated equilibrium sorption condition at the temperature of the yarn immediately prior to introduction into the hot crimping bath. In the case of a relatively water-insoluble but oil-soluble vaporizable liquid, such as heptane, the yarn is conditioned in contact either with the saturated vapor and/or with the liquid. The conditioned yarn is introduced quickly, while maintaining it free from tension and free to shrink, into a hot liquid crimping bath comprising a high boiling non-solvent for the yarn. The bath should have a temperature somewhat below the melting point of the yarn and at least 30° C. above the boiling point of the vaporizable liquid employed to condition the yarn. In the case of a continuous yarn, the rate at which the yarn is fed into the crimping bath may be 5% to 60% faster than the rate the yarn is withdrawn. Upon introduction into the crimping bath, the yarn immediately softens somewhat, and the vapor formed in situ from the vaporizable liquid is emitted steadily and rapidly as small bubbles at random from and/or through certain parts of the yarn surface. During emission of the vapors the yarn and the constituent filaments appear to gyrate in all directions and as the result, the filaments warp and bend irregularly to a crimped condition. Any strain remaining in the filaments after insertion of the crimp is

removed by permitting the yarn to remain in the crimping bath for a very short time after the vapors have apparently all been driven from the yarn. The total time during which the yarn 5 is permitted to remain in the crimping bath may vary widely depending upon the chemical composition of the yarn, the composition and method of the vaporizable substance with which the yarn is treated, the composition and temperature of the crimping bath, and possibly for other reasons. As a general rule, however, the total time of contact with the crimping bath should be not substantially less than  $\frac{1}{4}$  of a second and not more than 180 seconds. The crimped yarn is removed under substantially no tension from the crimping bath. The yarn is allowed to cool in a relaxed condition to room temperature in order to set the crimp to a condition that the crimped form is a normal stable one, substantially free from stress and strain.

The following examples illustrate certain specific applications of the invention, it being understood, of course, that they are not to be construed as being restrictive of the scope of the invention:

#### Example I

Untwisted, 10 denier per filament cellulose acetate yarn having a combined acetic acid content of about 54% is conditioned several days at room temperature in an atmosphere of high relative humidity (65% to 100% R. H.) until no further gain in moisture content is observed. The conditioned yarn is entered quickly but loosely into a light mineral oil bath which is held at a temperature between 180° C. and 220° C. Upon entrance into the oil bath, the yarn becomes softened and somewhat plastic and the moisture in and on the yarn is rapidly vaporized. The rapid and steady issuance of vapor at random from the surface of the yarn causes the filaments to warp and bend irregularly and a crimp results. After the moisture has been entirely driven from the yarn, the crimped yarn in its plastic condition is maintained in contact with the hot bath for a second or so longer in order to relieve all internal strains. In order to maintain the yarn in a loose condition in the oil bath, the feed rate of yarn into the bath is 10% to 25% greater than the rate of yarn take-off from the bath and in order to have sufficient time for driving off all the moisture and for heating the yarn slightly thereafter, the length of the bath is such as to give a yarn contact with the bath of approximately 2 to 3 seconds. After withdrawal from the bath, the yarn is allowed to cool in order to set the crimp. If desired, the oil is extracted from the yarn with suitable liquids such as toluene, trichlorethylene, or other dry cleaning agents. The oil may also be removed by scouring the yarn with  $\frac{1}{2}\%$  of Gardinol or soap solution at 75° C. to 85° C. After rinsing, the yarn is allowed to air dry. As measured on the dry yarn, the crimp inserted in the filaments by the oil bath amounts to 15 to 30 crimps per inch and not only is irregular as to form of the crimp, but also is distributed in a random manner along the length of the filaments. The crimped yarn is soft and bulky and has a desirable hand.

#### Example II

Instead of white mineral oil, olive oil heated to 190° to 200° C. may be used in the same manner as disclosed in Example I. If desired, the olive oil remaining on the yarn after the crimping treatment need not be completely removed,

but instead a residual amount, for instance, 2% to 4% or more, based on the weight of the dried yarn, may be left to serve as a finish during subsequent textile operations performed on the yarn.

*Example III*

A pile fabric, the pile of which consists largely of cellulose acetate fibers, is conditioned for several days at room temperature in an atmosphere having a humidity of nearly 100% R. H. until no further gain in moisture content is observed. The thus humidified fabric is immersed for about 2 seconds in a bath of white mineral oil held at a temperature between 180° and 220° C. After removing the fabric from the oil bath and allowing it to cool, the residual oil in the fabric is extracted by means of organic solvents such as toluene or dry cleaning fluid.

By virtue of the oil bath treatment, the fibers of the pile of the treated fabric are crimped and because of their crimped condition support each other to a large extent in an erect position and, in consequence, present more of a brush effect than similar but untreated fabric. The fabric also is more full and more crush-resistant than an untreated pile fabric.

*Example IV*

Cellulose acetate staple fibers of, for instance, 5.5 denier or 10 denier per filament are conditioned in a loose and open state over water at room temperature for several days so as to absorb as much moisture as possible without condensation of free water on the fibers. The moisture-containing staple fibers in a loose and fluffy physical condition are immersed for 2 to 4 seconds in a mineral oil bath that is held at a temperature of 180° to 220° C. The 2 to 4 seconds' contact of the fibers with the bath vaporizes off completely the moisture in the fibers and imparts a high degree of crimp. After withdrawal from the bath, the oil is removed from the staple fibers by centrifuging and subsequent extraction with organic solvents such as toluene or petroleum type solvents. The resulting crimped fibers possess a desirable appearance and feel.

*Example V*

Untwisted cellulose acetate yarn composed of a plurality of filaments, the filament denier of which is approximately 10, is immersed for several hours in heptane at room temperature. The thus conditioned yarn, while either wet with heptane or after all the free unabsorbed heptane has evaporated, is immersed for 2 to 4 seconds in hot mineral oil, which is held at a temperature of 150° to 210° C., and preferably at about 200° C. The oil treated yarn is subsequently handled as described in Example I and has a similar appearance.

*Example VI*

Untwisted viscose rayon yarn composed of a plurality of filaments, the filament denier of which is approximately 10, is immersed for several hours in water at room temperature. The wet yarn is passed through a pair of rubber squeeze rolls to remove the excess of water and then is entered rapidly in a hot mineral oil bath, the temperature of which is 190° to 220° C., and preferably 210° C. Substantially all the water in the yarn issues as steam which softens the yarn and warps the individual filaments thereof and yields a deep crimp therein. The length of time of contact of the yarn with the oil bath is

approximately 1 to 3 seconds, which permits the crimp to be inserted and permits also slight after-heating of the yarn to increase the stability of the crimp. After withdrawing the yarn without tension from the oil bath, the yarn is cooled and the oil is removed from the yarn in a manner described previously in the above examples. The resulting oil-free and dry viscose rayon yarn possesses a very definitely crimped condition and has a desirable appearance and hand.

*Example VII*

Untwisted gel viscose rayon yarn composed of a plurality of filaments, having a denier of about 10, which has been regenerated, desulfured, bleached, washed, but never dried, is submerged for 1 to 3 seconds in a mineral oil bath held at a temperature of 180° to 210° C. After withdrawal under no tension from the oil bath, the yarn is cooled and the oil is removed in the usual way. The resulting yarn is highly crimped and has an appearance similar to that described in Example VI.

The yarns may be impregnated or conditioned with volatilizable materials of many kinds and the specific selection will depend on factors such as the base material of the particular artificial yarn and the temperature of the crimping bath. The process will operate if the volatilizable or vaporizable material does not dissolve or swell the filaments excessively, or is employed in insufficient amounts to dissolve or swell the filaments excessively as the same is absorbed by the yarn, and may be driven off rapidly as a vapor while the filaments are in a softened or plastic condition. For instance, the volatilizable material may be a chemical compound which decomposes rapidly to vapors at the temperature of the crimping bath. In the case of liquid volatilizable conditioning agents, it is preferred that the liquid have a boiling point at least about 30° C. below the temperature of the crimping bath, and therefore at least about 30° C. below the melting point of the yarn treated. For instance, in the case of certain cellulose acetate yarns, it is desirable that the volatilizable liquid have a boiling point below 150°, and more preferably under 115° C. In the case of conditioning a thermoplastic yarn, such as cellulose acetate, with a volatilizable liquid such as water, it is preferred that the yarn be impregnated by contact with the vapors of the liquid rather than by direct contact with the liquid. In the case of water, the cellulose acetate yarn preferably is exposed at the temperature the yarn will have immediately prior to entrance into the crimping bath to an atmosphere of at least 30% R. H., and more preferably 95% to 100% R. H., until the equilibrium amount of moisture has been sorbed by the yarn. The cellulose acetate yarn, however, may be conditioned directly in contact with water, provided all water in excess of the equilibrium amount described in the preceding sentence is removed prior to immersion of the yarn in the crimping bath. In general, cellulose acetate yarn which is conditioned in an atmosphere the relative humidity of which is lower than 95% to 100% can be subjected to a higher temperature in the subsequent oil treatment than those conditioned at 100% R. H. In the case of conditioning liquids of the water-insoluble type, on the other hand, the crimp and the strength of the crimped cellulose acetate yarn is substantially the same, whether the absorption of the volatilizable material is accomplished by contact with the vapor or by contact directly with the

liquid. The following table discloses some volatilizable materials which can be used for conditioning cellulose acetate yarn and the results obtained when the yarn is conditioned by contact with the liquid and vapor form of the material. The table also describes the crimping bath temperature ranges which are suitable with each type of conditioning.

| Conditioning agent    | Crimping bath temperatures for yarn conditioned in the liquid | Crimping bath temperatures for yarn conditioned in vapor over the liquid |
|-----------------------|---------------------------------------------------------------|--------------------------------------------------------------------------|
| Isopropyl alcohol     | 115-200° C. (fibers slightly weak).                           | 115-200° C. (fibers strong).                                             |
| Methyl alcohol        | 100-200° C. (fibers weak)                                     | 115-185° C.                                                              |
| Carbon tetrachloride  | 135-200° C.                                                   | 135-210° C.                                                              |
| Toluene               | 150-210° C.                                                   | 175-210° C.                                                              |
| Benzene               | 150-200° C.                                                   | 150-200° C.                                                              |
| Heptane               | 165-215° C.                                                   | 165-215° C.                                                              |
| Acetic acid           | Dissolves yarn.                                               | 140-175° C.                                                              |
| 80% ethylene glyc. l. | do                                                            | 175-210° C.                                                              |
| 20% acetone           | do                                                            | 170-200° C.                                                              |
| 80% acetone           | do                                                            | 170-200° C.                                                              |
| 20% water             | 120-140° C.                                                   | 180-220° C.                                                              |
| Water                 |                                                               |                                                                          |

In such cases where vapors are best employed for conditioning, the yarn may be passed through a chamber filled with the vapors generated by heating the liquid. For instance, instead of conditioning cellulose acetate yarn over liquid water at room temperature for several days, the 30 yarn may be passed through a chamber into which water vapors are driven by elevating the temperature of the water. It is necessary in the use of the water vapors at elevated temperature to prevent condensation of liquid water on the 35 cellulose acetate yarn if it is planned to use a high crimping bath temperature.

The optimum amount of volatilizable material held by the yarn depends upon the base composition of the yarn and the crimping bath temperature used in driving out the volatile material. Cellulose acetate can best be conditioned, for example, by allowing it to absorb an equilibrium amount of moisture from an atmosphere of 95% to 100% R. H. at room temperature immediately after which the yarn is immersed in a hot oil crimping bath at a temperature of 180° to 220° C.

Liquid materials other than mineral oil may be used as the heating media of the crimping bath. The prime requisites for such a liquid material are that it should be substantially inert to the yarn treated, i. e., it should not swell, dissolve, or attack the yarn treated; it should not be unduly volatile at the temperature of treatment; it should not dissolve the vapor liberated from the yarn to any appreciable extent at the temperature of treatment; and it should be easily removed from the yarn after the yarn treatment. Accordingly, the choice of the material for the bath will depend largely upon the composition and type of yarn being treated and the temperature to be employed for the crimping. Bearing such factors in mind, the selection may be made from such materials as chlorinated diphenyl, chlorinated naphthalene, diphenyl, ethyl sebacate, olive oil, corn oil, castor oil, cottonseed oil, mineral oil, and metallic baths such as Wood's metal or mercury.

The temperature of the crimping treatment 70 may vary from approximately 115° C. to 250° C., or even wider, depending upon the kind of volatile material absorbed by the fibers before treatment in the hot bath and also upon the chemical nature of the yarn. In general, it is necessary 75

in the case of thermoplastic yarn that the temperature of the crimping bath be somewhat below the melting point of the yarn and at least 30° C. higher than the boiling point of the volatilizable or vaporizable conditioning material. In the particular case of cellulose acetate yarn, the lower the combined acetic acid content, the higher may the temperature of the crimping bath be, since the melting point of the yarn is somewhat higher and since the yarn may tolerate more moisture. Cellulose acetate yarn having a combined acetic acid content of 51.2% can be successfully crimped at 240° C.

The manner in which the conditioned yarns are 15 subjected to the hot bath treatment is extremely important. In the crimping bath it is necessary to secure an extremely rapid heat transfer between the heating medium and the yarn in order to produce the vapors in situ and emit the same 20 as small bubbles in a steady, rapid rate, but at random, from the surface of the yarn. Generally, the conditioned textile yarn is immersed quickly and passed through the hot oil crimping bath while maintained free from any tension and, therefore free to shrink, and withdrawn from the bath under little, if any, tension. In the case of 25 conditioned fibers such as staple lengths, it is important that they be placed loosely in the bath and in an open condition, so that they are in a position to shrink and crimp freely. The time of contact with the bath, as above described, is generally about  $\frac{1}{4}$  of a second to 180 seconds. It is desirable to have the yarn in contact with the oil bath for a sufficient period to insert the desired degree of crimp, but it is undesirable to have the yarn in contact with the bath too long, as such promotes a weakening, embrittlement, 30 discoloration, and charring of the yarn. It is also preferred to maintain the yarn in contact with the crimping bath for a sufficient period of time to not only drive off substantially all the volatilizable material, but also to after-heat for a very short time to remove any strained condition.

The most desirable manner of removing the 35 crimping medium, after the treatment, especially if an oil bath is employed, is to extract the oil or oily material with toluene or a petroleum fraction such as dry cleaner's liquid, which will dissolve the oil or oily substance and not affect the crimped yarn. Boil-off methods with soap or Gardinol (sodium salts of higher fatty alcohol sulfates) may be utilized, but the efficiency of oil removal is not so good as that obtained by the 40 organic solvent extraction method.

After the crimping medium has been removed, it is desirable to twist the crimped yarn to a degree commensurate with the yarn denier as is well known in the art. For many purposes such as for instance, the use of yarn in a warp, it is 45 highly desirable to size the twisted yarn with a warp size. In many such instances, it will be necessary to resort to sizing due to the fact that the yarn is bulky and provides a rough surface in contrast to the smooth rayon and silk yarn. Such rough crimped yarns abrade very easily and 50 tear readily unless properly sized. Any suitable sizing solution which is used in the art for sizing bulky threads to permit their use in textile operations may be employed.

In the above specification, reference has been 55 to cellulose acetate yarn as the thermoplastic artificial yarn. It will, of course, be recognized that the invention may also be applied to secure crimped yarns composed of other thermoplastic

maintaining the same free from tension, with a liquid non-solvent for said filaments, said liquid having a sufficiently elevated temperature to quickly volatilize said volatilizable material, and cause said filaments to crimp while in contact therewith, said volatilizable material having a boiling point at least 30° C. below the temperature of said liquid non-solvent.

4. The method of producing threads, yarns, fabrics, and like structures comprising filaments exhibiting deep, irregular crimps without substantially weakening the filaments which comprises applying to such structures comprising artificial filaments a volatilizable material, and then contacting said structures, while maintaining the same free from tension, with a liquid non-solvent for said filaments, said liquid having a temperature below the melting point of said structures but said temperature being sufficiently elevated to quickly volatilize said volatilizable material and cause said filaments to crimp while in contact therewith, said volatilizable material having a boiling point at least 30° C. below the temperature of said liquid non-solvent.

5. The method of producing threads, yarns, fabrics, and like structures comprising filaments exhibiting deep, irregular crimps without substantially weakening the filaments which comprises applying to such structures comprising artificial filaments vapors of a volatilizable material, and then contacting said structures, while maintaining the same free from tension, with a liquid non-solvent for said filaments, said liquid having a sufficiently elevated temperature to quickly volatilize said volatilizable material and cause said filaments to crimp while in contact therewith.

6. The method of producing threads, yarns, fabrics, and like structures comprising filaments exhibiting deep, irregular crimps without substantially weakening the filaments which comprises applying to such structures comprising artificial thermoplastic filaments vapors of a volatile material, and then contacting said structures, while maintaining the same free from tension, with a liquid non-solvent for said filaments, said liquid having a sufficiently elevated temperature to quickly volatilize said volatile material and cause said filaments to crimp while in contact therewith.

7. The method of producing threads, yarns, fabrics, and like structures comprising filaments exhibiting deep, irregular crimps without substantially weakening the filaments which comprises applying to such structures comprising artificial thermoplastic cellulosic filaments vapors of a volatilizable material, and then contacting said structures, while maintaining the same free from tension, with a liquid non-solvent for said filaments, said liquid having a sufficiently elevated temperature to quickly volatilize said volatilizable material and cause said filaments to crimp while in contact therewith.

8. The method of producing threads, yarns, fabrics, and like structures comprising filaments exhibiting deep, irregular crimps without substantially weakening the filaments which comprises applying to such structures comprising cellulose acetate filaments vapors of a volatilizable material, and then contacting said structures, while maintaining the same free from tension, with a liquid non-solvent for said filaments, said liquid having a sufficiently elevated temperature to quickly volatilize said volatilizable material and

cause said filaments to crimp while in contact therewith.

9. The method of producing threads, yarns, fabrics, and like structures comprising filaments exhibiting deep, irregular crimps without substantially weakening the filaments which comprises applying to such structures comprising artificial filaments vapor of a volatilizable material, and then contacting said structures, while maintaining the same free from tension, with a liquid non-solvent for said filaments, said liquid having a temperature below the melting point of said structures but said temperature being sufficiently elevated to quickly volatilize said volatilizable material and cause said filaments to crimp while in contact therewith.

10. The method of producing threads, yarns, fabrics, and like structures comprising filaments exhibiting deep, irregular crimps without substantially weakening the filaments which comprises applying to such structures comprising artificial filaments vapors of a volatilizable material, and then contacting said structures, while maintaining the same free from tension, with a liquid non-solvent for said filaments, said liquid having a temperature below the melting point of said structures but said temperature being sufficiently elevated to quickly volatilize said volatilizable material and cause said filaments to crimp while in contact therewith, said volatilizable material having a boiling point at least 30° C. below the temperature of said liquid non-solvent.

11. The method of producing threads, yarns, fabrics, and like structures comprising filaments exhibiting deep, irregular crimps without substantially weakening the filaments which comprises subjecting such structures comprising artificial filaments to an atmosphere having a relative humidity of at least 30%, until the moisture content of the structures comes to equilibrium, and then contacting said structures, while maintaining the same free from tension, with a liquid non-solvent for said filaments, said liquid having a sufficiently elevated temperature to quickly volatilize said moisture content of the structures and cause said filaments to crimp while in contact therewith.

50 12. The method of producing threads, yarns, fabrics, and like structures comprising filaments exhibiting deep, irregular crimps without substantially weakening the filaments which comprises subjecting such structures comprising artificial thermoplastic filaments to an atmosphere  
55 60 having a relative humidity of at least 30%, until the moisture content of the structures comes to equilibrium, and then contacting said structures, while maintaining the same free from tension, with a liquid non-solvent for said filaments, said liquid having a sufficiently elevated temperature to quickly volatilize said moisture content of the structures and cause said filaments to crimp while in contact therewith.

63 13. The method of producing threads, yarns, fabrics, and like structures comprising filaments exhibiting deep, irregular crimps without substantially weakening the filaments which comprises subjecting such structures comprising artificial thermoplastic cellulosic filaments to an atmosphere having a relative humidity of at least 30%, until the moisture content of the structures comes to equilibrium, and then contacting said structures, while maintaining the same free from tension, with a liquid non-solvent for said filaments, said liquid having a

70

75

materials such as cellulose acetate propionates, cellulose acetate butyrate, and other simple and mixed aliphatic acid esters of cellulose; as well as methyl cellulose, ethyl cellulose, propyl cellulose, butyl cellulose, and other organic ethers of cellulose; as well as yarns composed of vinyl acetate resins, vinyl acetal resins, vinyl chloride-vinyl acetate interpolymer resins, and other vinyl resins. Obviously, also the artificial materials to be crimped may contain within reason plasticizers, pigments, dyes, and other modifiers. Additionally, while perhaps of less interest, the invention may be applied to other cellulosic artificial yarns such as the regenerated cellulose type derived in the viscose and cuprammonium process. Because regenerated cellulose yarn is not thermoplastic, certain slight changes may be made in the process of the invention as compared to cellulose acetate yarn. For instance, in the case of regenerated cellulose yarn, the temperatures of the crimping bath can be increased considerably in many cases. Likewise, the specific choice of the volatilizable material may be somewhat different from that for cellulose acetate yarn. Additionally, the regenerated cellulose yarn in the case of water, can be humidified by exposure to a moist atmosphere or it may be soaked directly in water and the excess liquid water removed by shaking and the yarn crimped in the hot oil bath at a temperature of 180° to 220° C. All these slight differences, however, are considered to be well within the province of one skilled in the art.

The filament denier of the cellulose acetate yarn, as well as regenerated cellulose rayon yarn, has a very definite effect on the degree of crimp obtained. It has been found that filaments of heavy denier showed a most pronounced crimp. For instance, the degree of crimp of a 10 denier filament is greater than that of the 5.5 denier which, in turn, is greater than that of a 3 denier filament.

In the above specification any reference to an untwisted yarn is meant to include yarn having a very slight twist, for example, not more than two turns per inch whereby to hold the filaments together, as well as yarn having no twist. The term "yarn" in the present specification is intended to include yarn of continuous length and composed of individual continuous filaments, or yarn in which some of the filaments have been cut, or yarn cut to form filaments of staple length or other obvious modifications. The term "crimp" as used in the present specification is meant to include crimps, curls, undulations or other abrupt bends in the filaments and/or yarns.

By means of the present method a decided and accentuated crimp is imparted to the straight filaments and at the same time, all strains are relieved and the crimped filaments are set in their new and crimped form in a state in which the crimped form is normal and stable, while the straight condition is abnormal. The crimped yarns are thus put into a condition wherein more force is necessary to pull them out to a straight condition than necessary with filaments curled by mechanical or similar methods. The crimped yarns obtained in accordance with my methods disclosed herein are lofty in appearance and show a greater resistance to crushing than yarns curled by mechanical means. The yarns possess a relatively large number of fine and irregularly placed undulations or crimps per inch of length so that the yarns show good covering power and the fabrics produced therefrom show

a very definite and desirable depth and lofty hand.

It will be understood that the crimping process of the present invention may be combined with other methods of crimping to produce crimped filaments, threads, and the like having a composite crimp. Thus, in addition to imparting crimp according to the novel procedure described above, a further crimp can be imparted which may be either of a greater or less degree than the crimp which has been imparted by the oil crimping procedure. In following this modification, it is preferred that the second crimp be greater in degree, that is, less crimps per inch than the crimps produced by the oil crimping process. The oil crimping process of this invention can be supplemented, for example, by passing the yarn after it has been crimped by the oil crimping process, and preferably before the oil has been removed and while the yarn is still hot, through a crimping device such as is illustrated in Stone et al., Patent No. 1,973,581, issued September 11, 1934. Fabrics produced from yarns crimped in this manner have more fullness and bulk than fabrics composed of yarn which has been subjected only to the oil crimping process. It is understood, of course, that in this modification of the invention, reference to crimping with oil is illustrative and that in place of oil, the other equivalents of oil mentioned in this specification may, of course, be used.

Since it is obvious that many changes and modifications can be made in the above-detailed description without departing from the nature and spirit of the invention, it is to be understood that the invention is not to be limited except as set forth in the appended claims.

I claim:

1. The method of producing threads, yarns, fabrics, and like structures comprising filaments exhibiting deep, irregular crimps without substantially weakening the filaments which comprises applying to such structures comprising artificial thermoplastic filaments a volatilizable material, and then contacting said structures, while maintaining the same free from tension, with a liquid non-solvent for said filaments, said liquid having a sufficiently elevated temperature to quickly volatilize said volatilizable material, and cause said filaments to crimp while in contact therewith, said volatilizable material having a boiling point at least 30° C. below the temperature of said liquid non-solvent.

2. The method of producing threads, yarns, fabrics, and like structures comprising filaments exhibiting deep, irregular crimps without substantially weakening the filaments which comprises applying to such structures comprising artificial thermoplastic cellulosic filaments a volatilizable material, and then contacting said structures, while maintaining the same free from tension, with a liquid non-solvent for said filaments, said liquid having a sufficiently elevated temperature to quickly volatilize said volatilizable material, and cause said filaments to crimp while in contact therewith, said volatilizable material having a boiling point at least 30° C. below the temperature of said liquid non-solvent.

3. The method of producing threads, yarns, fabrics, and like structures comprising filaments exhibiting deep, irregular crimps without substantially weakening the filaments which comprises applying to such structures comprising cellulose acetate filaments a volatilizable material, and then contacting said structures, while

sufficiently elevated temperature to quickly volatilize said moisture content of the structures and cause said filaments to crimp while in contact therewith.

14. The method of producing threads, yarns, fabrics, and like structures comprising filaments exhibiting deep, irregular crimps without substantially weakening the filaments which comprises subjecting such structures comprising cellulose acetate filaments to an atmosphere having a relative humidity of at least 30%, until the moisture content of the structures comes to equilibrium, and then contacting said structures, while maintaining the same free from tension, with a liquid non-solvent for said filaments, said liquid having a sufficiently elevated temperature to quickly volatilize said moisture content of the structures and cause said filaments to crimp while in contact therewith.

15. The method of producing threads, yarns, fabrics, and like structures comprising filaments exhibiting deep, irregular crimps without substantially weakening the filaments which comprises subjecting such structures comprising artificial filaments to an atmosphere having a relative humidity of at least 30%, until the moisture content of the structures comes to equilibrium, and then contacting said structures, while maintaining the same free from tension, with a liquid non-solvent for said filaments, said liquid having a temperature below the melting point of said structures but said temperature being sufficiently elevated to quickly volatilize said moisture content of said structures and cause said filaments to crimp while in contact therewith.

16. The method of producing threads, yarns, fabrics, and like structures comprising filaments exhibiting deep, irregular crimps without substantially weakening the filaments which comprises subjecting such structures comprising artificial filaments to an atmosphere having a relative humidity of at least 30%, until the moisture content of the structures comes to equilibrium, and then contacting said structures, while maintaining the same free from tension, with an oil which is substantially inert to said filaments, said oil having a sufficiently elevated temperature to quickly volatilize said moisture content of the structures.

17. The method of producing threads, yarns, fabrics, and like structures comprising filaments exhibiting deep, irregular crimps without substantially weakening the filaments which comprises subjecting such structures comprising artificial thermoplastic filaments to an atmosphere having a relative humidity of at least 30%, until the moisture content of the structures comes to equilibrium, and then contacting said structures, while maintaining the same free from tension, with an oil which is substantially inert to said filaments, said oil having a sufficiently elevated temperature to quickly volatilize said moisture content of the structures.

18. The method of producing threads, yarns, fabrics, and like structures comprising filaments exhibiting deep, irregular crimps without substantially weakening the filaments which comprises subjecting such structures comprising artificial thermoplastic cellulosic filaments to an atmosphere having a relative humidity of at least 30%, until the moisture content of the structures comes to equilibrium, and then contacting said structures, while maintaining the same free from tension, with an oil which is

substantially inert to said filaments, said oil having a sufficiently elevated temperature to quickly volatilize said moisture content of the structures.

19. The method of producing threads, yarns, fabrics, and like structures comprising filaments exhibiting deep, irregular crimps without substantially weakening the filaments which comprises subjecting such structures comprising cellulose acetate filaments to an atmosphere having a relative humidity of at least 30%, until the moisture content of the structures comes to equilibrium, and then contacting said structures, while maintaining the same free from tension, with an oil which is substantially inert to said filaments, said oil having a sufficiently elevated temperature to quickly volatilize said moisture content of the structures.

20. The method of producing threads, yarns, fabrics, and like structures comprising filaments exhibiting deep, irregular crimps without substantially weakening the filaments which comprising subjecting such structures comprising artificial filaments to an atmosphere having a relative humidity of at least 30%, until the moisture content of the structures comes to equilibrium, and then contacting said structures, while maintaining the same free from tension, with an oil which is substantially inert to said filaments, said oil having a temperature below 25 the melting point of said structures but said temperature being sufficiently elevated to quickly volatilize said moisture content of said structures.

21. The method of producing threads, yarns, fabrics, and like structures comprising filaments exhibiting deep, irregular crimps without substantially weakening the filaments which comprises subjecting such structures comprising artificial filaments to an atmosphere having a relative humidity of between 95% and 100% until 35 the moisture content of the structures comes to equilibrium and then immersing said structures, while maintaining the same free from tension, into a bath of oil which is substantially inert to 40 said structures, said oil bath having a sufficiently elevated temperature to quickly volatilize said 45 moisture content of the structures.

22. The method of producing threads, yarns, fabrics, and like structures comprising filaments exhibiting deep, irregular crimps without substantially weakening the filaments which comprises subjecting such structures comprising artificial thermoplastic filaments to an atmosphere having a relative humidity of between 95% and 100% until the moisture content of the structures comes to equilibrium and then immersing said structures, while maintaining the same free from tension, into a bath of oil which is substantially inert to said structures, said oil bath having a sufficiently elevated temperature to quickly volatilize said moisture content of the structures.

23. The method of producing threads, yarns, fabrics, and like structures comprising filaments exhibiting deep, irregular crimps without substantially weakening the filaments which comprises subjecting such structures comprising artificial thermoplastic cellulosic filaments to an atmosphere having a relative humidity of between 95% and 100% until the moisture content of the structures comes to equilibrium and then immersing said structures, while maintaining the same free from tension, into a bath of oil which is substantially inert to said structures, said oil bath having a sufficiently elevated temperature

to quickly volatilize said moisture content of the structures.

24. The method of producing threads, yarns, fabrics, and like structures comprising filaments exhibiting deep, irregular crimps without substantially weakening the filaments which comprises subjecting such structures comprising cellulose acetate filaments to an atmosphere having a relative humidity of between 95% and 100% until the moisture content of the structures comes to equilibrium and then immersing said structures, while maintaining the same free from tension, into a bath of oil which is substantially inert to said structures, said oil bath having a sufficiently elevated temperature to quickly 15 volatilize said moisture content of the structures.

25. The method of producing threads, yarns, fabrics, and like structures comprising filaments exhibiting deep, irregular crimps without substantially weakening the filaments which comprises subjecting such structures comprising artificial filaments to an atmosphere having a relative humidity of between 95% and 100% until the moisture content of the structures comes to equilibrium and then immersing said 25

structures, while maintaining the same free from tension, into a bath of oil which is substantially inert to said structures, said oil bath having a temperature below the melting point of said 5 structures but said temperature being sufficiently elevated to quickly volatilize said moisture content of said structures.

26. The method of producing threads, yarns, fabrics, and like structures comprising filaments exhibiting deep, irregular crimps without substantially weakening the filaments which comprises subjecting such structures comprising artificial filaments to an atmosphere having a relative humidity of between 95% and 100% 10 until the moisture content of the structures comes to equilibrium and then immersing said structures, while maintaining the same free from tension, into a bath of oil which is substantially inert to said structures, said oil bath having a sufficiently elevated temperature to quickly 15 volatilize said moisture content of the structures, and maintaining the structures in contact with said bath until after all of the moisture has been volatilized therefrom.

HERON G. FINZEL.